# EUROPEAN PATENT SPECIFICATION

(11) **EP 1 416 599 B1**
(45) Date of publication and mention of the grant of the patent: **19.05.2010**
(21) Application number: 03256898.2
(22) Date of filing: 31.10.2003
(51) Int. Cl.: H01T 13/39, H01T 21/02

(54) **Spark plug and method for manufacturing the same**
Zündkerze und ihr Herstellungsverfahren
Bougie d'allumage et sa méthode de fabrication

(30) Priority: 01.11.2002 JP 2002320379
(43) Date of publication of application: 06.05.2004
(73) Proprietor: NGK SPARK PLUG CO., LTD, Mizuho-ku Nagoya-shi Aichi (JP)
(72) Inventor: Torii, Kazuyoshi, Mizuho-ku, Nagoya Aichi (JP); Teramura, Hideki, Mizuho-ku, Nagoya Aichi (JP); Kato, Tomoaki, Mizuho-ku, Nagoya Aichi (JP); Musasa, Mamoru, Mizuho-ku, Nagoya Aichi (JP)
(74) Representative: Nicholls, Michael John

(56) References cited:
- JP-A- 2001 244 042
- US-B1- 6 346 766

## Description

The present invention relates to a spark plug and the method for manufacturing the same.

Japanese Patent Application Laid-Open (*kokai*) No. 2001-244042 will be referred to herein as Patent Document 1. Patent Document 1 describes a conventionally known spark plug. This spark plug includes a tubular metallic shell. A tubular insulator is fixed in the metallic shell in such a manner as to extend in the axial direction of the metallic shell and such that the opposite ends of the insulator protrude from corresponding opposite ends of the metallic shell. A center electrode extends in the axial direction of the metallic shell such that the distal end of the center electrode protrudes from the distal end of the insulator, and the rear end of the center electrode is fixed in the insulator. Meanwhile, one end of a ground electrode is fixed to the metallic shell, and the other end portion of the ground electrode, together with the center electrode, forms a discharge gap therebetween. Each of the center electrode and the ground electrode includes an electrode base metal, which is an Ni alloy or the like such as Inconel (registered trademark) 600, and a chip provided on the electrode base metal at a position for forming the discharge gap and formed of a spark erosion resistant material such as an Ir-containing Pt alloy.

The center electrode of this spark plug is manufactured as follows. First there is formed a chip which includes a flange portion and a protrusion protruding from a first face of the flange portion. A second face of the chip opposite the protrusion is laser welded to a joint face of the electrode base metal located on the side toward the discharge gap, thereby forming the center electrode. At this time, a weld portion is formed in such a manner as to penetrate into the electrode base metal and the flange portion of the chip.

In this spark plug, the diameter of the flange portion of the chip is greater than that of the protrusion of the chip. Thus, as compared with the case of an ordinary columnar chip, a weld portion is formed over a wide range. Since a weld portion is formed in such a manner as to penetrate into the flange portion and the electrode base metal, there can be prevented a reduction in the diameter of a weld zone, which would otherwise result from spattering of the electrode base metal induced by laser welding. Thus, this spark plug can ensure the joining strength between the electrode base metal and the chip.

However, Patent Document 1, which discloses the above-described conventional spark plug, merely specifies that the weld portion be present over a certain distance or more as measured inward from the outer circumference of the flange portion of the chip. Thus, depending on the chip shape, difficulty may be encountered in ensuring the joining strength between the electrode base metal and the chip. For example, in the case where an employed chip includes a flange portion and a columnar protrusion, and the diameter of the protrusion is relatively large, a weld portion is formed only in the vicinity of the outer circumference of the flange portion, and thus the weld portion is not present in a large area at a central part of the flange portion. In such a case, sufficient joining strength between the electrode base metal and the chip fails to be ensured, and difficulty is encountered in maintaining the durability of the spark plug over a long term.

Also in the prior art, US 6,346,766 B1 discloses a spark plug according to the precharacterizing portion of the independent claims.

The present invention has been accomplished in view of the above-mentioned problems involved in the conventional spark plug, and an object of the invention is to provide a spark plug whose joining strength between an electrode base metal and a chip is reliably ensured, as well as to provide a method for manufacturing the same.

The present invention provides a method for manufacturing a spark plug which comprises a tubular metallic shell, a tubular insulator extending in an axial direction of the metallic shell and fixed in the metallic shell with opposite ends of the insulator protruding from corresponding opposite ends of the metallic shell, a center electrode extending in the axial direction of the metallic shell and fixed in the insulator with a distal end of the center electrode protruding from a distal end of the insulator and with a rear end of the center electrode fixed in the insulator, and a ground electrode with one end of the ground electrode fixed to the metallic shell and with the other end portion of the ground electrode and the center electrode forming a discharge gap therebetween, and in which at least either one of the center electrode and the ground electrode comprises an electrode base metal and a chip provided on the electrode base metal at a position for forming the discharge gap and formed of a spark erosion resistant material, the method comprising:
a first step of providing the chip which comprises a flange portion and a protrusion protruding from a first face of the flange portion;
a second step for tentatively joining, through resistance welding, a second face of the flange portion opposite the protrusion to a joint face of the electrode base metal of at least either one of the center electrode and the ground electrode, the joint face being located on a side toward the discharge gap; and
a third step for laser-welding the flange portion to the joint face such that a weld portion is formed between the electrode base metal and the chip to reach points on the second face of the flange portion, the points being located inward of corresponding intersections of the second face of the flange portion and imaginary extension lines of generatrices (generating lines) of a side surface of the protrusion.

According to the method for manufacturing a spark plug of the present invention, in the first step, the chip comprising the flange portion and the protrusion protruding from the first face of the flange portion is provided (for example by being manufactured). Next, in the second step, the second face of the flange portion is tentatively joined, through resistance welding, to the joint face of the electrode base metal of at least either one of the center electrode and the ground electrode, the joint face being located on the side toward the discharge gap. In the third step, the flange portion is laser-welded to the joint face of the electrode base metal. The laser welding is performed such that the weld portion is formed between the electrode base metal and the chip to reach points on the second face of the flange portion, the points being inward of corresponding intersections of the second face of the flange portion and imaginary extension lines of generatrices of the side surface of the protrusion. In the case where the protrusion of the chip assumes the shape of a cylinder, a prism, a circular cone, a pyramid, a frustum of a cone, or a frustum of a pyramid, the generatrices are lines extending on the side surface of the protrusion and capable of forming a common plane together with the axis of the protrusion. Thus, there can be prevented a problem that the weld portion is not present in a large area at a central part of the flange portion. Therefore, the flange portion is reliably joined to the joint face of the electrode base metal.

Thus, the method for manufacturing a spark plug of the present invention can ensure sufficient joining strength between the electrode base metal and the chip.

The method for manufacturing a spark plug of the present invention allows the joint face to be located on the electrode base metal of the ground electrode on the side toward the discharge gap. In other words, the method can be applied not only to the case of welding the chip to the electrode base metal of the center electrode, but also to the case of welding the chip to the electrode base metal of the ground electrode, which requires higher welding strength.

Preferably, in the method for manufacturing a spark plug of the present invention, when D represents the maximum distance between the intersections of the second face of the flange portion and imaginary extension lines of generatrices of the side surface of the protrusion, the weld portion is present in such a manner as to extend to a distance D/5 or more inward of the intersections as measured on the second face. The results of a test conducted by the present inventors have revealed that this feature ensures reliable joining of the flange portion and the joint face of the electrode base metal.

Preferably, in the method for manufacturing a spark plug of the present invention, in the first step, there is provided a plate-like intermediate member having a melting point or linear expansion coefficient falling between that of the electrode base metal and that of the chip, and having a face larger than the second face of the flange portion; and in the second step, the intermediate member is provided between the joint face and the chip. During the course of laser irradiation, employment of such an intermediate member provides good compatibility between the intermediate member and the electrode base metal and that between the intermediate member and the chip and reduces the difference in thermal stress to be induced between the intermediate member and the electrode base metal and that between the intermediate member and the chip. Therefore, separation hardly arises between the intermediate member and the electrode base metal and between the intermediate member and the chip.

Preferably, in the second step, after the intermediate member is tentatively joined to the joint face through resistance welding, the second face of the flange portion is tentatively joined to the intermediate member through resistance welding. This prevents movement of the intermediate member and the chip during the course of laser welding, thereby reliably welding the electrode base metal and the chip.

Preferably, in the method for manufacturing a spark plug of the present invention, when the joint face is located on the electrode base metal of the ground electrode on the side toward the discharge gap, the chip is welded to the ground electrode while the ground electrode is bent away from the distal end of the center electrode. Since this avoids imposition of restrictions on the angle of laser irradiation, the chip can be welded to the ground electrode at the optimum angle of laser irradiation.

The present invention provides a spark plug comprising a tubular metallic shell, a tubular insulator extending in an axial direction of the metallic shell and fixed in the metallic shell with opposite ends of the insulator protruding from corresponding opposite ends of the metallic shell, a center electrode extending in the axial direction of the metallic shell and fixed in the insulator with a distal end of the center electrode protruding from a distal end of the insulator and with a rear end of the center electrode fixed in the insulator, and a ground electrode with one end of the ground electrode fixed to the metallic shell and with the other end portion of the ground electrode and the center electrode forming a discharge gap therebetween, at least either one of the center electrode and the ground electrode comprising an electrode base metal and a chip provided on the electrode base metal at a position for forming the discharge gap and formed of a spark erosion resistant material,
wherein the chip comprises a flange portion and a protrusion protruding from a first face of the flange portion; a second face of the flange portion opposite the protrusion is tentatively joined, through resistance welding, to a joint face of the electrode base metal of at least either one of the center electrode and the ground electrode, the joint face being located on a side toward the discharge gap; and the flange portion is laser-welded to the joint face such that a weld portion is formed between the electrode base metal and the chip to reach points on the second face of the flange portion, the points being located inward of corresponding intersections of the second face of the flange portion and imaginary extension lines of generatrices of a side surface of the protrusion.

In the spark plug of the present invention, the chip comprises the flange portion and the protrusion, and laser welding is performed such that the weld portion is formed between the electrode base metal and the chip to reach points on the second face of the flange portion, the points being located inward of corresponding intersections of the second face of the flange portion and imaginary extension lines of generatrices of the side surface of the protrusion. Thus, there can be prevented a problem that the weld portion is not present in a large area at a central part of the flange portion. Therefore, the flange portion is reliably joined to the joint face of the electrode base metal, whereby the joining strength between the electrode base metal and the chip can be ensured, and the durability of the spark plug can be maintained over a long term.

Preferably, the weld portion contains components of the chip in an amount of 20% by mass to 80% by mass. According to the results of a test conducted by the present inventors, when the weld portion contains components of the chip in an amount less than 20% by mass or in excess of 80% by mass, the electrode base metal and the chip are unlikely to be compatible with each other, and a great difference arises in thermal stress to be induced between the electrode base metal and the chip, potentially resulting in a failure to ensure the joining strength between the electrode base metal and the chip. By contrast, when the weld portion contains components of the chip in an amount of 20% by mass to 80% by mass, the electrode base metal and the chip are compatible with each other, and the difference in thermal stress to be induced between the electrode base metal and the chip is small, whereby the joining strength between the electrode base metal and the chip can be readily ensured.

Particularly preferably, the weld portion contains components of the chip in an amount of 30% by mass to 60% by mass. This reliably ensures the joining strength between the electrode base metal and the chip.

An embodiment of the invention will now be described, by way of example only, with reference to the accompanying drawings in which:-
Fig. 1 relates to the embodiment and shows a process diagram of a method for manufacturing a spark plug;
Fig. 2 relates to the embodiment and shows a side view of a chip;
Fig. 3 relates to the embodiment and shows a side view of an intermediate member in the process of resistance welding;
Fig. 4 relates to the embodiment and shows a side view of the chip and the intermediate member in the process of resistance welding;
Fig. 5 relates to the embodiment and shows a side view of the chip and the intermediate member in the process of laser welding;
Fig. 6 relates to the embodiment and shows a center electrode or a ground electrode as viewed after laser welding;
Fig. 7 relates to the embodiment and shows a partially enlarged side view of a spark plug;
Fig. 8 relates to the embodiment and shows a partially enlarged side view of the spark plug;
Fig. 9 relates to the embodiment and shows a partially sectional side view of the spark plug; and
Fig. 10 relates to the embodiment and shows side views of other chips.
Reference numerals are used to identify items shown in the drawings as follows:
60: metallic shell
62: insulator
30: center electrode
40: ground electrode
1: chip
1 a: protrusion
1b: flange portion
2: intermediate member
3: weld portion
32, 42: joint face
S 10: first step
S20: second step
S30: third step

A spark plug and a method for manufacturing the same according to an embodiment of the present invention and a test for the spark plug and the method will be described with reference to Figs. 1 to 10.

### Embodiment

First, as shown in Fig. 1, in first step S10, a chip 1 is manufactured from a spark erosion resistant material, which is an Ir alloy containing at least any one of 1% by mass to 20% by mass Rh, 1% by mass to 10% by mass Pt, 1% by mass to 5% by mass Y₂O₃, and 1% by mass to 20% by mass Ni, or a Pt alloy containing at least any one of 20% by mass to 60% by mass Rh, 10% by mass to 40% by mass Ir, and 1% by mass to 20% by mass Ni. When the chip 1 is to be attached to both of a center electrode 30 and a ground electrode 40 (see Fig. 9), either the chips 1 of the same material or the chips 1 of different materials may be used. As shown in Fig. 2, the chip 1 includes a flange portion 1b and a protrusion 1 a protruding from a first face 1c of the flange portion 1b. The flange portion 1b assumes the shape of a disk and has a diameter L of 1 mm and a thickness of 0.2 mm. The protrusion 1a assumes a cylindrical shape and has a diameter R of 0.6 mm and a thickness of 0.5 mm.

As shown in Fig. 3, an intermediate member 2 is manufactured from an Ir alloy containing 40% by mass Ni. The intermediate member 2 assumes the shape of a disk and has a diameter L of 1.2 mm and a thickness of 0.2 mm.

In second step S20 shown in Fig. 1, as shown in Fig. 3, the intermediate member 2 is tentatively joined to the center electrode 30 through resistance welding. The center electrode 30 uses Inconel (registered trademark) 600, which is an Ni alloy, as an electrode base metal and has a diameter of 2.5 mm. For the tentative joining, first, the intermediate member 2 is placed on a joint face 32 of the center electrode 30, the joint face 32 facing a discharge gap. Then, a first electric resistance welding machine 50 is applied to the intermediate member 2. A predetermined current is applied to the first electric resistance welding machine 50 while a predetermined pressure is applied to the intermediate member 2, thereby tentatively joining the intermediate member 2 to the center electrode 30 through resistance welding.

Subsequently, as shown in Fig. 4, the flange portion 1b of the chip 1 is placed on the intermediate member 2, which is tentatively joined to the center electrode 30. A second electric resistance welding machine 60 is applied to the first face 1c of the flange portion 1b. A predetermined current is applied to the second electric resistance welding machine 60 while a predetermined pressure is applied to the first face 1 c. Notably, the second electric resistance welding machine 60 assumes such a structure as not to come into contact with the distal end face of the chip 1, whereby the distal end face of the chip 1 is free of any influence of the resistance welding. Thus, a second face 1 d of the flange portion 1b is tentatively joined to the intermediate member 2 through resistance welding, whereby the intermediate member 2 and the chip 1 are tentatively joined to the center electrode 30.

Next, in third step S30 shown in Fig. 1, as represented by the arrow of Fig. 5, a laser beam is irradiated so as to weld the flange portion 1b of the chip 1 to the joint face 32 of the center electrode 30. The laser welding is performed such that, as shown in Fig. 6, when D represents the maximum distance between the intersections of the second face 1d of the flange portion 1b and imaginary extension lines of generatrices extending on the side surface of the cylindrical protrusion 1a and capable of forming a common plane together with the axis of the protrusion 1a, and a represents the distance of the deepest point of a weld portion 3 as measured on the second face 1d from the intersection, a is D/5 or more. This allows the weld portion 3 to contain components of the chip 1 in an amount of 30% by mass to 60% by mass. Notably, in the present embodiment, D is equal to the diameter R of the protrusion 1.

Subsequently, as shown in Fig. 9, the center electrode 30 is fitted into an insulator 62 such that the distal end of the center electrode 30 protrudes from the insulator 62; and a terminal 63 is inserted into the insulator 62 to be located on the rear side of the center electrode 30. The resultant assembly is fitted into a metallic shell 60.

In fourth step S40 shown in Fig. 1, as shown in Fig. 9, the ground electrode 40, which is welded to the metallic shell 60 beforehand, is prepared. As in the case of the center electrode 30, the ground electrode 40 uses Inconel (registered trademark) 600, which is an Ni alloy, as an electrode base metal and has a width of 2.5 mm. As shown in Fig. 7 or 8, the ground electrode 40 is bent away from the distal end of the center electrode 30.

As shown in Fig. 3, the intermediate member 2 is tentatively joined to the ground electrode 40 through resistance welding. For the tentative joining, first, the intermediate member 2 is placed on a joint face 42 of the ground electrode 40, the joint face 42 facing the discharge gap. Then, the first electric resistance welding machine 50 is applied to the intermediate member 2. A predetermined current is applied to the first electric resistance welding machine 50 while a predetermined pressure is applied to the intermediate member 2, thereby tentatively joining the intermediate member 2 to the ground electrode 40 through resistance welding.

Subsequently, as shown in Fig. 4, the flange portion 1b of the chip 1 is placed on the intermediate member 2, which is tentatively joined to the ground electrode 40. The second electric resistance welding machine 60 is applied to the first face 1c of the flange portion 1b. A predetermined current is applied to the second electric resistance welding machine 60 while a predetermined pressure is applied to the first face 1c, thereby tentatively joining the second face 1d of the flange portion 1b to the intermediate member 2 through resistance welding. Thus, the intermediate member 2 and the chip 1 are tentatively joined to the ground electrode 40.

Next, in fifth step S50 shown in Fig. 1, as represented by the arrow of Fig. 5, a laser beam is irradiated so as to weld the flange portion 1b of the chip 1 to the joint face 42 of the ground electrode 40. The laser welding is performed such that, as shown in Fig. 6, when D represents the maximum distance between the intersections of the second face 1d of the flange portion 1b and imaginary extension lines of generatrices extending on the side surface of the cylindrical protrusion 1a and capable of forming a common plane together with the axis of the protrusion 1a, and a represents the distance of the deepest point of the weld portion 3 as measured on the second face 1d from the intersection, a is D/5 or more. This allows the weld portion 3 to contain components of the chip 1 in an amount of 30% by mass to 60% by mass. Notably, in the present embodiment, D is equal to the diameter R of the protrusion 1.

Subsequently, as shown in Figs. 7 and 8, the end portion of the electrode base metal of the ground electrode 40 to which the chip 1 has been welded is bent back toward the center electrode 30. Thus, the spark plug shown in Fig. 9 is obtained.

According to the method for manufacturing a spark plug of the present embodiment, in relation to the maximum distance D between the intersections of the second face 1d of the flange portion 1b and imaginary extension lines of generatrices extending on the side surface of the cylindrical protrusion 1a and capable of forming a common plane together with the axis of the protrusion 1a, the weld portion 3 is present in such a manner as to extend to a distance D/5 or more inward of the intersections as measured on the second face. Thus, there can be prevented a problem that the weld portion 3 is not present in a large area at a central part of the flange portion 1b. Therefore, the flange portion 1b is reliably joined to the joint face 32 (42) of the electrode base metal.

According to the method for manufacturing a spark plug of the present embodiment, the intermediate member 2 has a melting point and a linear expansion coefficient falling between those of the electrode base metal and those of the chip 1; thus, during the course of laser irradiation, good compatibility is established between the intermediate member 2 and the electrode base metal and between the intermediate member 2 and the chip 1, and the difference in thermal stress to be induced between the intermediate member 2 and the electrode base metal and that between the intermediate member 2 and the chip 1 can be reduced. Therefore, separation hardly arises between the intermediate member 2 and the electrode base metal and between the intermediate member 2 and the chip 1.

According to the method for manufacturing a spark plug of the present embodiment, after the intermediate member 2 is tentatively joined to the joint face 32 (42) through resistance welding, the second face 1d of the flange portion 1b is tentatively joined to the intermediate member 2 through resistance welding; thus, movement of the intermediate member 2 and the chip 1 during the course of laser welding can be prevented, whereby the electrode base metal and the chip 1 can be reliably welded together.

Therefore, the method for manufacturing a spark plug of the present embodiment can reliably ensure the joining strength between the electrode base metal and the chip 1.

According to the method for manufacturing a spark plug of the present embodiment, the chip 1 is welded to the ground electrode 40 while the ground electrode 40 is bent away from the distal end of the center electrode 30. Since this avoids imposition of restrictions on the angle of laser irradiation, the chip 1 can be welded to the ground electrode 40 at the optimum angle of laser irradiation.

As shown in Fig. 9, the thus-obtained spark plug includes the tubular metallic shell 60. The tubular insulator 62 is fixed in the metallic shell 60 in such a manner as to extend in the axial direction of the metallic shell 60 and such that the opposite ends of the insulator 62 protrude from corresponding opposite ends of the metallic shell 60. The center electrode 30 extends in the axial direction of the metallic shell 60 such that the distal end of the center electrode 30 protrudes from the distal end of the insulator 62, and the rear end of the center electrode 30 is fixed in the insulator 62. Meanwhile, one end of the ground electrode 40 is fixed to the metallic shell 60, and the other end portion of the ground electrode 40, together with the center electrode 30, forms a discharge gap therebetween. The chips 1 are provided on the center electrode 30 and the ground electrode 40, respectively, in opposition to each other while maintaining a discharge gap therebetween.

In this spark plug, the chip 1 includes the flange portion 1b and the protrusion 1a. The chip 1 is laser-welded to the electrode base metal such that the weld portion 3 is formed between the electrode base metal and the chip 1 and reaches points on the second face 1d of the flange portion 1b, the points being located inward of corresponding intersections of the second face 1d of the flange portion 1b and imaginary extension lines of generatrices extending on the side surface of the cylindrical protrusion 1a and capable of forming a common plane together with the axis of the protrusion 1 a. Thus, there can be prevented a problem that the weld portion 3 is not present in a large area at a central part of the flange portion 1b. Therefore, the flange portion 1b is reliably joined to the joint face 32 (42) of the electrode base metal, whereby the joining strength between the electrode base metal and the chip 1 can be ensured, and the durability of the spark plug can be maintained over a long term.

In this spark plug, since the weld portion 3 contains components of the chip 1 in an amount of 30% by mass to 60% by mass, the electrode base metal and the chip 1 are compatible with each other, and the difference in thermal stress to be induced between the electrode base metal and the chip 1 is small, whereby the joining strength between the electrode base metal and the chip 1 can be readily ensured.

### Test

A test for verifying the effect of the method for manufacturing a spark plug of the present embodiment was carried out. First, the chips 1 and the intermediate members 2 were manufactured by use of alloys similar to those of the embodiment and in shapes similar to those of the embodiment. Four types of the chips 1 were manufactured as follows: as shown in Fig. 6, when D represents the maximum distance (equal to the diameter R of the protrusion 1; hereinafter called the "diameter R of the protrusion 1") between intersections of the second face 1d of the flange portion 1b and imaginary extension lines of generatrices extending on the side surface of the cylindrical protrusion 1a and capable of forming a common plane together with the axis of the protrusion 1a, D is 0.6 mm, 0.8 mm, 1.0 mm, and 1.2 mm. The diameter of the flange portion 1b is 0.4 mm greater than the diameter R of the protrusion 1 of each type.

Each of the chips 1 was laser-welded, in a manner similar to that of the embodiment, to an electrode base metal that was an alloy similar to that used to form the center electrode 30 and the ground electrode 40 of the embodiment. The test was conducted for the following two cases: the intermediate member 2 was used as in the case of the embodiment; and, without use of the intermediate member 2, the chip 1 was directly laser-welded to the electrode base metal.

The test conditions are described below. The chip 1 was laser-welded to the electrode base metal as follows: when a represents the distance of the deepest point (hereinafter, called "penetration") of the weld portion 3 as measured on the second face 1 d from the intersection between the second face 1d of the flange portion 1b and an imaginary extension line of a generatrix of the side surface of the protrusion 1a, the weld portion 3 of a predetermined penetration a was formed for each type of the chip 1. The weld portion was heated for two minutes by use of a burner and was then allowed to cool at the room temperature for one minute. After this cycle was repeated for 50 hours, the weld portion was examined for the length of an oxide scale. The oxide scale refers to a defect induced by a difference in thermal stress; specifically, a crack observed on the cross section of the chip 1 or exfoliation of the chip 1. The burner temperature was 900°C and 950°C.

Tables 1 to 4 show the test results. Table 1 shows the test results for a diameter R of the protrusion 1 of 0.6 mm; Table 2 shows the test results for a diameter R of the protrusion 1 of 0.8 mm; Table 3 shows the test results for a diameter R of the protrusion 1 of 1.0 mm; and Table 4 shows the test results for a diameter R of the protrusion 1 of 1.2 mm. In Tables 1 to 4, "o" indicates that the length b of an oxide scale is less than L/3, where L is the diameter of the flange portion 1b; "Δ" indicates that the length b of an oxide scale is equal to or greater than L/3 and less than L/2; and "×" indicates that the length b of an oxide scale is equal to or greater than L/2.

**Table 1**

| | | | | | |
|---|---|---|---|---|---|
| D=0.6mm | | | | | |

| Intermediate member | Temperature (°C) | Penetration a (mm) | | | |
|---|---|---|---|---|---|
| | | 0.10 | 0.12 | 0.15 | 0.18 |
| Absent | 900 | × | o | o | o |
| | 950 | × | o | o | o |
| Present | 900 | Δ | o | o | o |
| | 950 | × | o | o | o |

**Table 2**

| | | | | | |
|---|---|---|---|---|---|
| D=0.8mm | | | | | |

| Intermediate member | Temperature (°C) | Penetration a (mm) | | | |
|---|---|---|---|---|---|
| | | 0.10 | 0.13 | 0.16 | 0.20 |
| Absent | 900 | × | Δ | o | o |
| | 950 | × | × | o | o |
| Present | 900 | Δ | Δ | o | o |
| | 950 | × | Δ | o | o |

**Table 3**

| | | | | | |
|---|---|---|---|---|---|
| D = 1.0 mm | | | | | |

| Intermediate member | Temperature (°C) | Penetration a (mm) | | | |
|---|---|---|---|---|---|
| | | 0.10 | 0.15 | 0.20 | 0.25 |
| Absent | 900 | × | × | o | o |
| | 950 | × | × | o | o |
| Present | 900 | × | Δ | o | o |
| | 950 | × | × | o | o |

**Table 4**

| | | | | | |
|---|---|---|---|---|---|
| D = 1.2 mm | | | | | |

| Intermediate member | Temperature (°C) | Penetration a (mm) | | | |
|---|---|---|---|---|---|
| | | 0.10 | 0.15 | 0.20 | 0.25 |
| Absent | 900 | × | × | Δ | o |
| | 950 | × | × | × | o |
| Present | 900 | × | Δ | Δ | o |
| | 950 | × | × | × | o |

As is apparent from Tables 1 to 4, when the penetration a is equal to or greater than D/5, all of the test results are evaluated as "o," indicating that the length b of a scale is less than L/3. The test results reveal that, when the penetration a is equal to or greater than D/5, the joining strength between the electrode base metal and the chip 1 can be reliably ensured.

The manufacturing method of the embodiment can employ chips in various shapes; for example, chips 71 to 73 shown in Figs. 10(a) to 10(c). In the case of the chip 71 shown in Fig. 10(a), a protrusion 71a has a taper surface. In the case of the chip 72 shown in Fig. 10(b), a flange portion 72b has a taper surface. In the case of the chip 73 shown in Fig. 10(c), a protrusion 73a has a taper surface, and the diameter of a bottom surface 73c of the protrusion 73a is equal to that of the flange portion 72b. Even when these chips 71 to 73 are used, the effect of the present invention can be yielded.

According to the manufacturing method of the embodiment, both of the protrusion and the flange portion assume a circular shape. However, the present invention is not limited thereto. A polygonal (e.g., triangular or quadrangular) chip may be used. Also, the protrusion and the flange portion do not necessarily assume the same shape.

According to the manufacturing method of the embodiment, the center electrode and the ground electrode use Inconel (registered trademark) as an electrode base metal. However, the present invention is not limited thereto. The electrode base metal may be, for example, Ni, an Ni alloy, Fe, or an Fe alloy.

## Claims

1. A method for manufacturing a spark plug which comprises a tubular metallic shell (60), a tubular insulator (62) extending in an axial direction of the metallic shell (60) and fixed in the metallic shell (60) with opposite ends of the insulator (62) protruding from corresponding opposite ends of the metallic shell (60), a center electrode (30) extending in the axial direction of the metallic shell (60) and fixed in the insulator (62) with a distal end of the center electrode (30) protruding from a distal end of the insulator (62) and with a rear end of the center electrode (30) fixed in the insulator (62), and a ground electrode (40) with one end of the ground electrode (40) fixed to the metallic shell (60) and with the other end portion of the ground electrode (40) and the center electrode (30) forming a discharge gap therebetween, and in which at least one of the center electrode (30) and the ground electrode (40) comprises an electrode base metal and a chip (1) provided on the electrode base metal at a position for forming the discharge gap and formed of a spark erosion resistant material, **characterized in that** the method comprises:
a first step of providing the chip (1) which comprises a flange portion (1b) and a protrusion (1a) protruding from a first face (1c) of the flange portion;
a second step of tentatively joining, through resistance welding, a second face (1d) of the flange portion (1b) opposite the protrusion (1a) to a joint face (32/42) of the electrode base metal of at least either one of the center electrode (30) and the ground electrode (40), the joint face (32/42) being located on a side toward the discharge gap; and
a third step of laser-welding the flange portion (1b) to the joint face (32/42) such that a weld portion (3) is formed between the electrode base metal and the chip to reach points on the second face (1d) of the flange portion (1b), the points being located inward of corresponding intersections of the second face (1d) of the flange portion (1b) and imaginary extension lines of generatrices of a side surface of the protrusion (1a).

2. A method for manufacturing a spark plug as described in claim 1, wherein the joint face (32/42) is located on the electrode base metal of the ground electrode (40) on a side toward the discharge gap.

3. A method for manufacturing a spark plug as described in claim 2, wherein, when D represents a maximum distance between the intersections, the weld portion (3) is present in such a manner as to extend to a distance D/5 or more inward of the intersections as measured on the second face.

4. A method for manufacturing a spark plug as described in any one of claims 1 to 3, wherein the first step further comprises providing a plate-like intermediate member (2) having at least one of a melting point and linear expansion coefficient falling between that of the electrode base metal and that of the chip (1), and having a face larger than the second face (1d) of the flange portion (1b); and
the second step further comprises providing the intermediate member (2) between the joint face (32/42) and the chip (1).

5. A method for manufacturing a spark plug as described in claim 4, wherein the second step further comprises, after the intermediate member (2) is tentatively joined to the joint face (32/42) through resistance welding, tentatively joining the second face (1d) of the flange portion (1b) to the intermediate member (2) through resistance welding.

6. A method for manufacturing a spark plug as described in any one of claims 1 to 5, further comprising locating the joint face (32/42) on the electrode base metal of the ground electrode (40) on a side toward the discharge gap, and welding the chip (1) to the ground electrode (40) while the ground electrode (40) is bent away from the distal end of the center electrode (30).

7. A spark plug comprising a tubular metallic shell (60), a tubular insulator (62) extending in an axial direction of the metallic shell (60) and fixed in the metallic shell (60) with opposite ends of the insulator (62) protruding from corresponding opposite ends of the metallic shell (60), a center electrode (30) extending in the axial direction of the metallic shell (60) and fixed in the insulator (62) with a distal end of the center electrode (30) protruding from a distal end of the insulator (62) and with a rear end of the center electrode (30) fixed in the insulator (62), and a ground electrode (40) with one end of the ground electrode (40) fixed to the metallic shell (60) and with the other end portion of the ground electrode (40) and the center electrode (30) forming a discharge gap therebetween, at least one of the center electrode (30) and the ground electrode (40) comprising an electrode base metal and a chip (1) provided on the electrode base metal at a position for forming the discharge gap and formed of a spark erosion resistant material, **characterized in that**:
the chip (1) comprises a flange portion (1b) and a protrusion (1a) protruding from a first face (1c) of the flange portion (1b);
a second face (1d) of the flange portion (1b) opposite the protrusion (1a) is tentatively joined, through resistance welding, to a joint face (32/42) of the electrode base metal of at least either one of the center electrode (30) and the ground electrode (40), the joint face (32/42) being located on a side toward the discharge gap; and
the flange portion (1b) is laser-welded to the joint face (32/42) such that a weld portion (3) is formed between the electrode base metal and the chip (1) to reach points on the second face (1d) of the flange portion (1b), the points being located inward of corresponding intersections of the second face (1d) of the flange portion (1b) and imaginary extension lines of generatrices of a side surface of the protrusion (1a).

8. A spark plug as described in claim 7, wherein the weld portion (3) contains components of the chip (1) in an amount in the range of from 20% by mass to 80% by mass.

9. A spark plug as described in claim 8, wherein the weld portion (3) contains components of the chip (1) in an amount in the range of from 30% by mass to 60% by mass.

## Patentansprüche

1. Verfahren zum Herstellen einer Zündkerze, umfassend ein rohrförmiges metallisches Gehäuse (60), einen rohrförmigen Isolator (62), welcher sich in einer axialen Richtung des metallischen Gehäuses (60) erstreckt und in dem metallischen Gehäuse (60) befestigt ist, wobei gegenüberliegende Enden des Isolators (62) von den entsprechenden gegenüberliegenden Enden des metallischen Gehäuses (60) hervorstehen, eine Mittelelektrode (30), welche sich in der axialen Richtung des metallischen Gehäuses (60) erstreckt und in dem Isolator (62) befestigt ist, wobei ein distales Ende der Mittelelektrode (30) von einem distalen Ende des Isolators (62) hervorsteht und ein hinteres Ende der Mittelelektrode (30) in dem Isolator (62) befestigt ist, und eine Masseelektrode (40), wobei ein Ende der Masseelektrode (40) an dem metallischen Gehäuse (60) befestigt ist und der andere Endbereich der Masseelektrode (40) und die Mittelelektrode (30) einen Entladungsabstand dazwischen bilden, und in welcher zumindest eine der Mittelelektrode (30) und der Masseelektrode (40) ein Elektrodenbasismetall und einen Chip (1) umfasst, welcher auf dem Elektrodenbasismetall an einer Position zur Bildung des Entladungsabstands bereitgestellt ist und aus einem funkenerosionsresistentem Material gebildet ist, **dadurch gekennzeichnet, dass** das Verfahren umfasst:
einen ersten Schritt des Bereitstellens des Chips (1), welcher einen Flanschbereich (1 b) und einen von einer ersten Fläche (1 c) des Flanschbereichs hervorstehenden Vorsprung (1 a) umfasst;
einen zweiten Schritt des vorläufigen Verbindens mittels Widerstandsschweißen einer zweiten Fläche (1 d) des Flanschbereichs (1 b) gegenüber dem Vorsprung (1 a) mit einer Verbindungsfläche (32/42) des Elektrodenbasismetalls von zumindest einem der Mittelelektrode (30) und der Masseelektrode (40), wobei die Verbindungsfläche (32/42) auf einer in Richtung des Entladungsabstands weisenden Seite angeordnet ist; und
einen dritten Schritt des Laserschweißens des Flanschbereichs (1 b) an die Verbindungsfläche (32/42), so dass ein Schweißbereich (3) zwischen dem Elektrodenbasismetall und dem Chip ausgebildet wird, um Punkte auf der zweiten Fläche (1 d) des Flanschbereichs (1 b) zu erreichen, wobei die Punkte einwärts von entsprechenden Schnittpunkten der zweiten Fläche (1 d) des Flanschbereichs (1 b) und imaginären Verlängerungslinien von Erzeugenden einer Seitenoberfläche des Vorsprungs (1 a) angeordnet sind.

2. Verfahren zur Herstellung einer Zündkerze wie in Anspruch 1 beschrieben, wobei die Verbindungsfläche (32/42) auf dem Elektrodenbasismetall der Masseelektrode (40) auf einer in Richtung des Entladungsabstands weisenden Seite angeordnet ist.

3. Verfahren zur Herstellung einer Zündkerze wie in Anspruch 2 beschrieben, wobei, wenn D einen Maximalabstand zwischen den Schnittpunkten repräsentiert, der Schweißbereich (3) in solch einer Weise vorliegt, dass er sich bis zu einem Abstand D/5 oder mehr nach innen von den Schnittpunkten, gemessen auf der zweiten Fläche, erstreckt.

4. Verfahren zur Herstellung einer Zündkerze wie in einem der Ansprüche 1 bis 3 beschrieben, wobei der erste Schritt des Weiteren das Bereitstellen eines plattenartigen Zwischenelements (2) umfasst, welches zumindest eines eines Schmelzpunkts und linearen Expansionskoeffizienten aufweist, welche zwischen die des Elektrodenbasismetalls und die des Chips (1) fallen, und welches eine Fläche größer als die zweite Fläche (1 d) des Flanschbereichs (1 b) aufweist; und
der zweite Schritt des Weiteren das Bereitstellen des Zwischenelements (2) zwischen der Verbindungsfläche (32/42) und des Chips (1) umfasst.

5. Verfahren zur Herstellung einer Zündkerze wie in Anspruch 4 beschrieben, wobei der zweite Schritt des Weiteren umfasst, nachdem das Zwischenelement (2) mittels Widerstandsschweißen vorläufig mit der Verbindungsfläche (32/42) verbunden wurde, vorläufiges Verbinden der zweiten Fläche (1d) des Flanschbereichs (1 b) mit dem Zwischenelement (2) mittels Widerstandsschweißen.

6. Verfahren zur Herstellung einer Zündkerze wie in einem der Ansprüche 1 bis 5 beschrieben, des Weiteren umfassend das Anordnen der Verbindungsfläche (32/42) auf dem Elektrodenbasismetall der Masseelektrode (40) auf einer in Richtung des Entladungsabstands weisenden Seite und Schweißen des Chips (1) an die Masseelektrode (40) während die Masseelektrode (40) von dem distalen Ende der Mittelelektrode (30) weggebogen wird.

7. Zündkerze, umfassend ein rohrförmiges metallisches Gehäuse (60), einen rohrförmigen Isolator (62), welcher sich in einer axialen Richtung des metallischen Gehäuses (60) erstreckt und in dem metallischen Gehäuse (60) befestigt ist, wobei gegenüberliegende Enden des Isolators (62) von den entsprechenden gegenüberliegenden Enden des metallischen Gehäuses (60) hervorstehen, eine Mittelelektrode (30), welche sich in der axialen Richtung des metallischen Gehäuses (60) erstreckt und in dem Isolator (62) befestigt ist, wobei ein distales Ende der Mittelelektrode (30) von einem distalen Ende des Isolators (62) hervorsteht und ein hinteres Ende der Mittelelektrode (30) in dem Isolator (62) befestigt ist, und eine Masseelektrode (40), wobei ein Ende der Masseelektrode (40) an dem metallischen Gehäuse (60) befestigt ist und der andere Endbereich der Masseelektrode (40) und die Mittelelektrode (30) einen Entladungsabstand dazwischen bilden, wobei zumindest eine der Mittelelektrode (30) und der Masseelektrode (40) ein Elektrodenbasismetall und einen Chip (1) umfasst, welcher auf dem Elektrodenbasismetall an einer Position zur Bildung des Entladungsabstands bereitgestellt ist und aus einem funkenerosionsresistentem Material gebildet ist, **dadurch gekennzeichnet, dass**:
der Chip (1) einen Flanschbereich (1 b) und einen von einer ersten Fläche (1 c) des Flanschbereichs (1 b) hervorstehenden Vorsprung (1 a) umfasst;
eine zweite Fläche (1 d) des Flanschbereichs (1 b) gegenüber dem Vorsprung (1 a) mittels Widerstandsschweißen mit einer Verbindungsfläche (32/42) des Elektrodenbasismetalls von zumindest einem der Mittelelektrode (30) und der Masseelektrode (40) vorläufig verbunden ist, wobei die Verbindungsfläche (32/42) auf einer in Richtung des Entladungsabstands weisenden Seite angeordnet ist; und
der Flanschbereich (1 b) an die Verbindungsfläche (32/42) lasergeschweißt ist, so dass ein Schweißbereich (3) zwischen dem Elektrodenbasismetall und dem Chip (1) ausgebildet ist, um Punkte auf der zweiten Fläche (1 d) des Flanschbereichs (1 b) zu erreichen, wobei die Punkte einwärts von entsprechenden Schnittpunkten der zweiten Fläche (1 d) des Flanschbereichs (1 b) und imaginären Verlängerungslinien von Erzeugenden einer Seitenoberfläche des Vorsprungs (1 a) angeordnet sind.

8. Zündkerze wie in Anspruch 7 beschrieben, wobei der Schweißbereich (3) Komponenten des Chips (1) in einer Menge im Bereich von 20 Masse-% bis 80 Masse-% enthält.

9. Zündkerze wie in Anspruch 8 beschrieben, wobei der Schweißbereich (3) Komponenten des Chips (1) in einer Menge im Bereich von 30 Masse-% bis 60 Masse-% enthält.

## Revendications

1. Procédé pour fabriquer une bougie d'allumage qui comprend une enveloppe métallique tubulaire (60), un isolateur tubulaire (62) s'étendant dans une direction axiale de l'enveloppe métallique (60) et fixé dans l'enveloppe métallique (60) avec des extrémités opposées de l'isolateur (62) qui font saillie à partir d'extrémités opposées correspondantes de l'enveloppe métallique (60), une électrode centrale (30) s'étendant dans la direction axiale de l'enveloppe métallique (60) et fixée dans l'isolateur (62) avec une extrémité distale de l'électrode centrale (30) qui fait saillie à partir d'une extrémité distale de l'isolateur (62) et avec une extrémité arrière de l'électrode centrale (30) fixée dans l'isolateur (62), et une électrode de masse (40) avec une extrémité de l'électrode de masse (40) fixée à l'enveloppe métallique (60) et avec l'autre partie d'extrémité de l'électrode de masse (40) et l'électrode centrale (30) qui forment un espace de décharge entre elles, au moins l'une de l'électrode centrale (30) et de l'électrode de masse (40) comprenant un métal de base d'électrode et une pastille (1) disposée sur le métal de base d'électrode en une position permettant de former l'espace de décharge et constituée par un matériau résistant à l'érosion par les étincelles, **caractérisé en ce que** le procédé comprend :
une première étape consistant à disposer la pastille (1), qui comprend une partie de flasque (1b) et une saillie (1a) faisant saillie à partir d'une première face (1c) de la partie de flasque ;
une deuxième étape consistant à tenter de réunir, par soudage résistif, une deuxième face (1d) de la partie de flasque (1b) opposée à la saillie (1a) à une surface de réunion (32/42) du métal de base d'électrode d'au moins l'une ou l'autre de l'électrode centrale (30) et de l'électrode de masse (40), la face de réunion (32/42) étant située sur un côté dirigé vers l'espace de décharge ; et
une troisième étape consistant à souder au laser la partie de flasque (1b) à la face de réunion (32/42) de telle sorte qu'une partie de soudage (3) soit formée entre le métal de base d'électrode et la pastille, de façon à atteindre des points sur la deuxième face (1d) de la partie de flasque (1b), les points étant situés à l'intérieur d'intersections correspondantes de la deuxième face (1d) de la partie de flasque (1b) et de lignes d'extension imaginaires de génératrices d'une surface latérale de la saillie (1a).

2. Procédé pour fabriquer une bougie d'allumage selon la revendication 1, dans lequel la face de réunion (32/42) est située sur le métal de base d'électrode de l'électrode de masse (40) sur un côté dirigé vers l'espace de décharge.

3. Procédé pour fabriquer une bougie d'allumage selon la revendication 2, dans lequel, lorsque D représente une distance maximale entre les intersections, la partie de soudage (3) est présente de façon à s'étendre jusqu'à une distance de D/5 ou plus vers l'intérieur des intersections, mesurée sur la deuxième face.

4. Procédé pour fabriquer une bougie d'allumage selon l'une quelconque des revendications 1 à 3, dans lequel la première étape comprend de plus la disposition d'un élément intermédiaire en forme de plaque (2) ayant au moins l'un parmi un point de fusion et un coefficient de dilatation linéaire compris entre ceux du métal de base d'électrode et ceux de la pastille (1), et ayant une face plus grande que la deuxième face (1d) de la partie de flasque (1b) ; et
la deuxième étape comprend de plus la disposition de l'élément intermédiaire (2) entre la face de réunion (32/42) et la pastille (1).

5. Procédé pour fabriquer une bougie d'allumage selon la revendication 4, dans lequel la deuxième étape comprend de plus, après la tentative de réunion de l'élément intermédiaire (2) à la face de réunion (32/42) par soudage résistif, une tentative de réunion de la deuxième face (1d) de la partie de flasque (1b) à l'élément intermédiaire (2) par soudage résistif.

6. Procédé pour fabriquer une bougie d'allumage selon l'une quelconque des revendications 1 à 5, comprenant de plus la disposition de la face de réunion (32/42) sur le métal de base d'électrode de l'électrode de masse (40) sur un côté dirigé vers l'espace de décharge, et le soudage de la pastille (1) à l'électrode de masse (40) tandis que l'électrode de masse (40) est incurvée de façon à l'éloigner de l'extrémité distale de l'électrode centrale (30).

7. Bougie d'allumage comprenant une enveloppe métallique tubulaire (60), un isolateur tubulaire (62) s'étendant dans une direction axiale de l'enveloppe métallique (60) et fixé dans l'enveloppe métallique (60) avec des extrémités opposées de l'isolateur (62) qui font saillie à partir d'extrémités opposées correspondantes de l'enveloppe métallique (60), une électrode centrale (30) s'étendant dans la direction axiale de l'enveloppe métallique (60) et fixée dans l'isolateur (62) avec une extrémité distale de l'électrode centrale (30) qui fait saillie à partir d'une extrémité distale de l'isolateur (62) et avec une extrémité arrière de l'électrode centrale (30) fixée dans l'isolateur (62), et une électrode de masse (40) avec une extrémité de l'électrode de masse (40) fixée à l'enveloppe métallique (60) et avec l'autre partie d'extrémité de l'électrode de masse (40) et l'électrode centrale (30) qui forment un espace de décharge entre elles, au moins l'une de l'électrode centrale (30) et de l'électrode de masse (40) comprenant un métal de base d'électrode et une pastille (1) disposée sur le métal de base d'électrode en une position permettant de former l'espace de décharge et constituée par un matériau résistant à l'érosion par les étincelles, **caractérisée en ce que** :
la pastille (1) comprend une partie de flasque (1b) et une saillie (1a) faisant saillie à partir d'une première face (1c) de la partie de flasque (1b) ;
on tente de réunir, par soudage résistif, une deuxième face (1d) de la partie de flasque (1b), opposée à la saillie (la), à une face de réunion (32/42) du métal de base d'électrode d'au moins l'une ou l'autre de l'électrode centrale (30) et de l'électrode de masse (40), la face de réunion (32/42) étant située sur un côté dirigé vers l'espace de décharge ; et
la partie de flasque (1b) est soudée au laser à la face de réunion (32/42) de telle sorte qu'une partie de soudure (3) soit formée entre le métal de base d'électrode et la pastille (1) de façon à atteindre des points sur la deuxième face (1d) de la partie de flasque (1b), les points étant situés vers l'intérieur d'intersections correspondantes de la deuxième face (1d) de la partie de flasque (1b) et de lignes d'extension imaginaires de génératrices d'une surface latérale de la saillie (1a).

8. Bougie d'allumage selon la revendication 7, dans laquelle la partie de soudure (3) contient des composants de la pastille (1) sous une quantité située dans la plage comprise entre 20% en masse et 80% en masse.

9. Bougie d'allumage selon la revendication 8, dans laquelle la partie de soudure (3) contient des composants de la pastille (1) sous une quantité située .dans la plage comprise entre 30% en masse et 60% en masse.
